

Patented Nov. 2, 1926.

1,605,139

## UNITED STATES PATENT OFFICE.

SAMUEL H. PARRISH, OF CHICAGO, ILLINOIS, ASSIGNOR, BY DIRECT AND MESNE ASSIGNMENTS, TO S. H. PARRISH COMPANY, OF CHICAGO, ILLINOIS, A CORPORATION OF ILLINOIS.

DRIER.

No Drawing.

Application filed April 5, 1923. Serial No. 630,157.

106-310

My invention is more particularly designed for use in connection with the compositions for rendering paper transparent and increasing its electrical resistance. Such a composition is disclosed in a Patent No. 1,419,750 granted to me the 13th day of June, 1922. It is obviously desirable for the rapid handling of paper treated with the material in question, that it dries as rapidly as possible after the treatment in order that it may be rolled up or otherwise formed into a compact bulk without the layers sticking together. It is the purpose of the present invention to provide a drier which, when added to the composition of the patent or similar compositions, will cause the paper treated therewith to dry rapidly so that it may be properly handled commercially in large quantities.

I prepare the drier in the following manner; I first mix four (4) ounces of acetone, four (4) ounces of carbon-tetrachloride and approximately two (2) teaspoonfuls of commercial sodium silicate which normally contains about thirty per cent (30%) of sodium silicate and seventy per cent (70%) water. The precise proportions given are not essential as any of the above described components may be substantially varied without departing from my invention in its broader aspect. These materials are well stirred together until thoroughly mixed and dissolved and then permitted to stand over night and decanted to free the mixture from the sediment which forms, or the material may be strained through a close meshed filter; I separately dissolve four (4) ounces of a vegetable gum such as rosin but preferably bleached shellac in twelve (12) ounces of acetone or other known solvent thereof. After the gum has been thoroughly dissolved I let the mixture stand over night and then decant or strain it to free it of sediment. The two mixtures are then poured together and thoroughly stirred and

the resultant mixture is then ready to be added to the composition for rendering paper transparent and increasing its electrical resistance. The precise proportions of shellac or other gum to solvent are not material but those given have been found to be satisfactory.

The resultant mixture may be added to the patented composition in a wide range of proportions, depending upon the nature of the paper to be treated and the desired effect. For thin papers which dry more readily I have added to the patented composition one-quarter of its weight of drier and where thick papers are to be treated, I have added as much as one-half as much drier as composition to be dried. The most satisfactory amount for any particular paper can readily be determined by experiment. In case it is preferred that the paper dry more slowly, balsam gum may be added to the drier. I have added balsam in the proportion of one-twentieth by weight to the drier with good results but the proportion thereof may be varied within wide limits.

I have found that with such additions to the composition for making the paper transparent or insulating, the paper treated therewith dries in a few moments after the composition has been applied thereto so that the layers thereof will not adhere to each other, permitting the paper to be continuously unwound from a roll, treated with the composition and rolled up again at a relatively rapid speed without the adherence of the layers to each other.

I claim:

1. A drier for the purpose described comprising acetone, carbon-tetrachloride, sodium silicate, and shellac.
2. A drier for the purpose described comprising acetone, carbon-tetrachloride, sodium silicate, shellac and balsam.

SAMUEL H. PARRISH.